

[54] COLOR DIFFUSION TRANSFER DYE IMAGE-FORMING MATERIAL BINDER LAYERS CONTAINING A WATER-SOLUBLE CELLULOSE SALT

[75] Inventors: Peter O. Kliem, Weston; Jerome L. Reid, Wayland, both of Mass.

[73] Assignee: Polaroid Corporation, Cambridge, Mass.

[\*] Notice: The portion of the term of this patent subsequent to Dec. 12, 1989, has been disclaimed.

[22] Filed: Dec. 11, 1973

[21] Appl. No.: 423,669

[52] U.S. Cl. .... 96/73; 96/3; 96/29 D; 96/74; 96/77; 96/113

[51] Int. Cl. G03C 7/00; G03C 5/54; G03C 1/76; G03G 3/00

[58] Field of Search ..... 96/3, 29 D, 77, 99, 100, 96/73, 113, 74

[56]

#### References Cited

##### UNITED STATES PATENTS

|           |         |                     |         |
|-----------|---------|---------------------|---------|
| 2,357,590 | 9/1944  | Jaffe et al. ....   | 96/113  |
| 2,956,883 | 10/1960 | De Pauw et al. .... | 96/113  |
| 3,077,400 | 2/1963  | Rogers ....         | 96/29 D |
| 3,705,798 | 12/1972 | Kliem et al. ....   | 96/3    |

Primary Examiner—Norman G. Torchin  
Assistant Examiner—Richard L. Schilling  
Attorney, Agent, or Firm—Gerald L. Smith

[57]

#### ABSTRACT

Photographic products for forming diffusion transfer images, particularly multicolor transfer images, which products contain one or more gelatin-containing layers including the addition of a water-soluble cellulose salt.

4 Claims, 6 Drawing Figures



PATENTED SEP 9 1975

3,904,417

SHEET 1 OF 3





FIG. 3



FIG. 4



**COLOR DIFFUSION TRANSFER DYE  
IMAGE-FORMING MATERIAL BINDER LAYERS  
CONTAINING A WATER-SOLUBLE CELLULOSE  
SALT**

**BACKGROUND**

The present invention is directed to providing new and improved diffusion transfer-process photographic film units adapted to provide, as a function of the point-to-point degree of photoexposure, by diffusion transfer processing, a dye transfer image.

A number of photographic systems for forming images by diffusion transfer are well known in the art. Generally speaking, such systems comprise the steps of photoexposing a light-sensitive material, typically a light-sensitive silver halide layer, to form a developable image; contacting the thus exposed light-sensitive material with a photographic processing composition to develop said image and to form an imagewise distribution of mobile and diffusible image-forming constituents; and transferring this imagewise distribution, at least in part, by diffusion, to an image-receiving layer to impart thereto the desired transfer image. The image-receiving layer may be contained on a separate support, i.e., as a separate element, or in lieu thereof, the image-receiving layer and the photosensitive layer may be contained as a unitary product on the same support, e.g., as a laminar produce including the photosensitive layer, the image-receiving layer, and any other additional layers which may be desirable or necessary in the particular photographic system employed.

Black-and-white transfer images may be provided by the well known silver transfer system wherein a light-sensitive silver halide layer, e.g., a gelatino silver halide emulsion layer, is exposed and then developed with an aqueous alkaline processing composition including a silver halide developing agent and a silver halide solvent to form in terms of unexposed areas an imagewise distribution of a soluble silver complex which is then transferred, at least in part, by diffusion, to a silver-receptive stratum where it is reduced to impart thereto a positive silver transfer image.

Color transfer images may be obtained by various systems employing color image-providing materials which may be complete dyes or dye intermediates, e.g., color couplers. The color image-providing material may be initially insoluble or nondiffusible in the particular processing composition employed or it may be initially soluble or diffusible in the processing composition. In either instance, and in accordance with the particular image-forming mechanism employed, upon contacting the exposed photosensitive layer with the appropriate processing composition, an imagewise distribution of soluble and diffusible color image-providing material is formed and this imagewise distribution is then transferred, at least in part, by diffusion, to a superposed image-receiving layer, e.g., a dyeable stratum, to impart thereto a color transfer image. This image may be monochromatic or multicolor, depending upon the system employed, particularly whether two or more photosensitive layers and associated color image-providing material are so employed.

A particularly useful system for preparing color transfer images is that described and claimed in U.S. Pat. No. 2,983,606 employing as the color image-providing material a dye developer, i.e., a dye which is also a silver halide developing agent. In such a sys-

tem, an exposed silver halide layer containing a developable image is developed by contacting it with an aqueous alkaline solution containing a dye developer. The dye developer develops the exposed silver halide and is in turn oxidized to provide an oxidation product which is less mobile and diffusible than unreacted (un-oxidized) dye developer. An imagewise distribution of the unoxidized dye developer is then transferred, by diffusion, to a dyeable stratum to impart thereto a positive color transfer image.

Other color image-providing materials and systems employing them to form color transfer images, are also known in the art. By way of illustration, mention may be made of the materials and systems disclosed in the following U.S. Pat. Nos.: 2,647,049; 2,661,293; 2,698,244; 2,698,798; 2,802,735; 3,148,062; 3,227,550; 3,227,551; 3,227,552; 3,227,554; 3,243,294; 3,330,655; 3,347,671; 3,352,672; 3,364,022; 3,443,939; 3,443,940; 3,443,941; etc.

In any of the aforementioned systems monochromatic color transfer images may be obtained by employing a photographic product or film unit containing a single photosensitive layer which is exposed and then developed in the presence of one or, if desired, a mixture of color image-providing materials. Multicolor images may be obtained in the manner known in the art by employing a photographic product containing two or more selectively sensitized photosensitive layers each having associated therewith a color image-providing material of predetermined spectral absorption characteristics. A typical photographic product for preparing multicolor images comprises a photosensitive element comprising a blue-, a green- and a red-sensitive silver halide emulsion layer having associated therewith in the same or in a contiguous layer a yellow, a magenta and a cyan color image-providing material, respectively. Thus, a typical photographic product employing dye developers may comprise a support carrying, in order, a cyan dye developer layer, a red-sensitive silver halide emulsion layer, a magenta dye developer layer, a green-sensitive silver halide emulsion layer, a yellow dye developer layer, and a blue-sensitive silver halide emulsion layer. Photographic products contemplated for use in forming multicolor transfer images may, and preferably do contain interlayers disposed between the red-sensitive silver halide emulsion layer and the magenta dye developer [or other color image-providing material] layer and/or between the green-sensitive silver halide emulsion layer and the yellow dye developer. An additional or auxiliary layer may be, and preferably is, disposed over the blue-sensitive silver halide emulsion layer.

Common to all of these systems is a photographic product or film unit having one or more gel-containing layers. The gel-containing layer may be the light-sensitive layer or layers, e.g., a gelatino silver halide emulsion layer, the layer containing the color image-providing material, e.g., any of the dye developer layers previously described and/or the interlayers, auxiliary layer, etc. The dye developers employed may be incorporated with their associated silver halide emulsion layer or, in the preferred embodiment, in a separate layer behind the respective silver halide stratum. The developer is distributed in a film-forming natural, or synthetic, polymer, for example, gelatin, polyvinyl alcohol, and the like, adapted to be permeated by a chosen diffusion transfer fluid processing composition. To pro-

vide a more efficient and useful film unit product incorporating the above-outlined features, it is desirable to utilize "low-gel" systems. Such systems provide for significant reduction in the gelatin constituent of any layer or strata. The consequent lower strata thicknesses serve to improve diffusion transfer activity. Selective additives, for instance, those described in U.S. Pat. No. 3,705,798 have been found useful in deriving low gel systems. However, in some gelatin carried dye-developer strata, certain typical additives may tend to promote aggregating effects and the like.

#### SUMMARY OF THE INVENTION

The present invention is directed to new and improved negative/positive integral or multicomponent diffusion transfer process photographic film units adapted to provide, by diffusion transfer processing, a photographic color image reproduction as a function of the exposure of such film units to incident actinic radiation.

In one aspect, the photographic film unit of the invention provides for the improved performance of diffusion transfer process dye image-forming materials. This is achieved by providing with the dye dispersion, within an aqueous alkaline solution polymeric binder, a water-soluble cellulose salt. Preferably, this salt is selected as sodium cellulose sulfate.

In another aspect, the water-soluble cellulose salt may be incorporated with silver halide emulsion layers having associated therewith dye image-providing materials, or in each of discrete strata thereof.

The film unit assembly's construction employed in the practice of the present invention may comprise a film unit of the general type set forth in U.S. Pat. Nos. 3,415,644,-5 and -6; 3,473,925; 3,573,042,-3 and -4; 3,576,625 and -6; 3,594,164 and -5; 3,615,421; 3,620,724; 3,647,434,-5 and -7; 3,661,585; 3,672,890; and 3,689,262, and will include, disposed in a photosensitive element which contains a plurality of layers including, in predetermined order, two dimensionally stable layers at least one of which is transparent and intermediate said dimensionally stable layers, a plurality of layers including at least a dyeable polymeric layer and a photosensitive layer comprising a plurality of strata containing one or more photosensitive silver halide layers, each having associated therewith a diffusion transfer process dye image-forming material disposed within a polymeric binder and incorporating a water soluble cellulose salt. The unit also may contain means for providing a processing composition in contact with the photosensitive layers at a select location within the unit in dependence upon its particular structure.

#### BRIEF DESCRIPTION OF THE DRAWINGS

FIG. 1 is a perspective view, partially in section, showing a typical photographic film unit embodying the invention;

FIG. 2 is an exploded perspective view of the film unit of FIG. 1;

FIG. 3 is a somewhat schematic, longitudinal, sectional view of one embodiment of the film unit, the thickness of the materials being exaggerated for purposes of clarity of illustration;

FIG. 4 is a diagrammatic, enlarged, cross-sectional view of a portion of one embodiment of a film unit illustrating in detail the arrangement of layers of materials therewithin;

FIG. 5 is another schematic, longitudinal sectional view of another embodiment of the film unit, the thickness of materials and components being exaggerated for purposes of clarity of illustration; and

FIG. 6 is a diagrammatic, enlarged, cross-sectional view of a portion of the film unit of FIG. 5.

#### DETAILED DESCRIPTION

Reference is now made to FIGS 1 and 2 of the drawings wherein there is illustrated one film unit structure of a type which may embody the invention. The film unit, designated 10, generally includes dimensionally stable layers or sheets 12 and 14, and a rupturable container 16 holding a quantity of processing liquid 17. The two sheets and processing liquid include all of the materials and reagents required to produce a full-color photographic print as described by appropriate ones of the aforementioned patents.

The basic construction of the film unit 10 remains somewhat the same for unitary image producing systems which may be incorporated therewithin. For such structures, distinctions may be found in the nature of support sheets 12 and 14, that is, whether one or both are transparent, and the noted disposition of various layers and strata coated thereupon. As set forth in the earlier referenced patents, the structure of the film units may be designed for more or less typical operation wherein photosensitive and image receiving portions are joined for processing and separated thereafter following an interval of imbibition. In the particular embodiment shown in FIGS. 1 and 2, the photosensitive structure of the unit is exposed and the image is viewed through sheet 14 which, accordingly, is transparent.

In addition to sheets 12 and 14 and container 16, film unit 10 includes a mask or binding element 18 and a trapping element 20. Sheets 12 and 14 are secured in face-to-face relation at their lateral and trailing margins by binding element 18 as shown. Element 18 preferably is formed of a light opaque material.

Container 16 is of a type shown in U.S. Pat. No. 2,543,181 and is formed by folding a rectangular blank of a fluid-impervious sheet material medially and sealing the marginal sections of the blank to one another to form a cavity for containing processing liquid 17. The seal along the marginal section of the container adjacent sheets 12 and 14 is weaker than the end seals. Accordingly, upon the application of a predetermined compressive force to the walls of the container, there will be generated within the liquid a hydraulic pressure sufficient to separate the noted weaker seal so as to provide for the discharge of fluid 17 at a select location intermediate sheets 12 and 14. Container 16 is retained in place by appropriate portions of binder element 18.

In processing the film units shown, the unit is advanced, container 16 foremost, relative to and between a pair of pressure-applying members such as rolls (see FIG. 3). These members initially apply compressive pressure to the container to cause it to eject its liquid contents between sheets 12 and 14, then distribute the mass of liquid between the sheets toward the trailing ends thereof to form a layer of substantially uniform predetermined thickness which is continuous and at least co-extensive with the exposure opening defined by element 18. Trapping element 20 is incorporated within the structure to collect and retain excess processing liquid.

Looking to FIGS. 3 and 4, an embodiment for film unit 10 in which dimensionally stable sheet 14 is transparent and sheet 12 is opaque, is revealed in exaggerated detail. As shown more clearly in FIG. 4, the laminate structure incorporates photosensitive layers having a plurality of strata. For instance, the photosensitive strata includes, in order, cyan dye developer layer 24; red sensitive silver halide emulsion layer 26; an interlayer 28; magenta dye developer layer 30; green-sensitive silver halide emulsion layer 32; interlayer 34; yellow dye developer layer 36; blue-sensitive silver halide emulsion layer 38; auxiliary layer 40 which may contain an auxiliary silver halide developing agent; image-receiving layer 42 which may be a dyeable polymeric layer; spacer layer 44 and neutralizing layer 46. The latter layer is juxtaposed to transparent dimensionally stable sheet layer 14.

Supporting sheets or elements 12 and 14 may be formed from a variety of materials, for instance, paper base materials, ethylene glycol terephthalic acid; vinyl chloride polymers; polyvinyl acetate; polyamides; polymethacrylic acid; methyl and ethyl esters; cellulose derivatives, such as cellulose acetate, triacetate, nitrate, propionate, butyrate acetate or acetate butyrates; cross linked polyvinyl alcohol, and so forth.

The respective silver halide emulsion layers may comprise gelatino mixed silver halide emulsions, e.g., silver iodobromide emulsions, selectively sensitized as noted above.

The interlayers and/or the auxiliary layer may comprise gelatin or some other suitable material. For example, each of the two interlayers may comprise the coalescence of a synthetic polymeric latex and a composition which provides selective permeability thereto in accordance with the invention described in a now abandoned application for U.S. Patent by Avtges et al., Ser. No. 880,205, filed Nov. 26, 1969,

The dye developers are compounds which contain, in the same molecule, both the chromophoric system of a dye and also a silver halide developing function. By "a silver halide developing function" is meant a grouping adapted to develop exposed silver halide. A preferred silver halide development function is a hydroquinonyl group. Other suitable developing functions include ortho-dihydroxyphenyl and ortho- and para-amino substituted hydroxyphenyl groups. In general, the development function includes a benzenoid developing function, that is, an aromatic developing group which forms quinonoid quinone substances when oxidized.

The dye developers are preferably selected for their ability to provide colors that are useful in carrying out subtractive color photography, that is, the previously mentioned cyan, magenta and yellow. The dye developers employed may be incorporated in the respective silver halide emulsions or, in the illustrated embodiment, in a separate layer adjacent the respective silver halide stratum. The dye developers are distributed in a film-forming natural or synthetic polymer, for example, gelatin, polyvinyl alcohol, and the like, adapted to be permeated by the chosen diffusion transfer fluid processing composition.

The photosensitive layer or component of unit 10 for the instant or related structural embodiment would include layers 12, 24-40 and may be prepared, for example, by coating, in succession on a gelatin subbed

opaque cellulose triacetate film base, the following layers:

1. a layer of the cyan dye developer 1,4-bis-( $\beta$ -[hydroquinonyl- $\alpha$ -methyl]-ethylamino)5,8-dihydroxy-anthraquinone dispersed in gelatin and coated at a coverage of about 150 mgs./ft.<sup>2</sup> of dye and about 200 mgs./ft.<sup>2</sup> of gelatin;
2. a red-sensitive gelatino-silver iodobromide emulsion coated at a coverage of about 200 mgs./ft.<sup>2</sup> of silver and about 100 mgs./ft.<sup>2</sup> of gelatin;
3. a layer of gelatin coated at a coverage of about 200 mgs./ft.<sup>2</sup>;
4. a layer of the magenta dye developer 2-(p-[ $\beta$ -hydroquinonylethyl]-phenylazo)-4-isopropoxy-1-naphthol dispersed in gelatin and coated at a coverage of 70 mgs./ft.<sup>2</sup> of dye and about 100 mgs./ft.<sup>2</sup> of gelatin;
5. a green-sensitive gelatino-silver iodobromide emulsion coated at a coverage of about 100 mgs./ft.<sup>2</sup> of silver and 60 mgs./ft.<sup>2</sup> of gelatin;
6. a layer of gelatin coated at a coverage of about 150 mgs./ft.<sup>2</sup>;
7. a layer of the yellow dye developer 4-(p-[ $\beta$ -hydroquinonylethyl]-phenylazo)-3-(N-n-hexylcarboxamido)-1-phenyl-5-pyrazolone dispersed in gelatin and coated at a coverage of about 40 mgs./ft.<sup>2</sup> of dye and 50 mgs./ft.<sup>2</sup> of gelatin;
8. a blue-sensitive gelatino-silver iodobromide emulsion coated at a coverage of about 60 mgs./ft.<sup>2</sup> of silver and about 50 mgs./ft.<sup>2</sup> of gelatin; and
9. a layer containing 4'-methylphenyl hydroquinone dispersed in gelatin and coated at a coverage of about 10 mgs./ft.<sup>2</sup> of 4'-methylphenyl hydroquinone and about 30 mgs./ft.<sup>2</sup> of gelatin.

Where the structural embodiment of the photographic unit is one wherein the photosensitive and image receiving portions thereof are separated following an interval of imbibition, the image receiving portion may be one as described, for example, in U.S. Pat. No. 3,362,819.

In the embodiment of FIGS. 3 and 4, disclosed, for example, in the earlier referenced patents, including No. 3,415,644, a unitary or composite arrangement is provided wherein the processing composition 17 provided from container 16 is unidirectionally discharged intermediate auxiliary layer 40 and image receiving layer 42. A somewhat schematic representation for this geometry is revealed in FIG. 3, the figure also showing the forwardmost portion of container 16 being introduced between pressure applying rolls 50 and 52.

The unitary or composite film unit of the type shown in FIGS. 3 and 4, may be prepared by first successively coating layers 24-40 on support 12 in the manner described immediately above. Then transparent dimensionally stable sheet 14, for instance cellulose triacetate film base, may be coated, in succession, with the following illustrative layers:

1. the partial butyl ester of polyethylene/maleic anhydride copolymer prepared by refluxing, for 14 hours, 300 grams of high viscosity poly(ethylene/maleic anhydride), 140 grams of n-butyl alcohol and 1 cc. of 85% phosphoric acid to provide a polymeric acid layer approximately 0.75 mils. thick;
2. a solution of hydroxypropyl cellulose in water to provide a polymeric spacer layer approximately 0.075 mils. thick;

3. a 2:1 mixture, by weight, of polyvinyl alcohol and poly-4-vinylpyridine, at a coverage of approximately 600 mgs./ft.<sup>2</sup>, to provide a polymeric image-receiving layer approximately 0.40 mils. thick; and  
 4. then baking the element at 180°F. for 30 minutes and cooling.

The two components thus prepared may then be taped together in laminate form, for instance, by binder element 18 at their respective edges. Rupturable container 16 containing an aqueous alkaline processing solution 17 comprising:

| Water                                                                                                                                              | 100  | cc. | grams |
|----------------------------------------------------------------------------------------------------------------------------------------------------|------|-----|-------|
| Potassium hydroxide                                                                                                                                | 11.2 |     | grams |
| Hydroxyethyl cellulose (high viscosity) [commercially available from Hercules Powder Co., Wilmington, Delaware, under the trade name Natrasol 250] | 3.4  |     | grams |
| N-benzyl- $\alpha$ -picolinium bromide                                                                                                             | 1.5  |     | grams |
| Benzotriazole                                                                                                                                      | 1.0  |     | grams |
| Titanium dioxide                                                                                                                                   | 40.0 |     | grams |

may then be mounted on the leading edge of each of the laminates by pressure sensitive binding element 18 or other suitable means providing the above-noted necessary geometry for proper distribution of the fluid intermediate layers 40 and 42. Subsequent to the distribution of the processing solution, a multicolor dye transfer image formation at layer 42 may be viewed through transparent sheet 14 against a reflecting background, for instance, provided by the titanium dioxide constituent of the solution.

Turning to FIGS. 5 and 6, another film unit structure appropriate for the instant invention is illustrated. Described in detail in U.S. Pat. No. 3,594,164, film unit 60 assumes the general configuration of unit 10 shown in FIGS. 1 and 2, however, its laminar structure as well as the geometry of its dimensionally stable layers and processing fluid container are different. Film unit 60 comprises a rupturable container 62 retaining, prior to processing, aqueous alkaline solution 64, photosensitive laminate 66 including, in order, blue-sensitive silver halide emulsion layer 68 containing yellow dye developer appropriately dispersed within a gelatin carrier; interlayer 70; green-sensitive silver halide emulsion layer 74 containing magenta dye developer; interlayer 74; red-sensitive silver halide emulsion layer 76 containing cyan dye developer; opaque layer 78; image-receiving layer 80; spacer layer 82; neutralizing layer 84; dimensionally stable transparent layer 86 and dimensionally stable opaque sheet 88 (FIG. 5). Both layer 86 and sheet 88 preferably comprise processing composition impermeable flexible sheet material.

The composite may be provided with a binding member extending around, for example, the specified edges of the laminate, as illustrated in the figures. The binding member may comprise a pressure-sensitive tape, portions of which are revealed at 90 securing laminate elements together at the composite specified edges. Tape 90 will also act to maintain processing composition 64 intermediate sheet 88 and photosensitive laminate 66 upon application of compressive pressure to container 62 and distribution of its contents intermediate the stated elements. Under such circumstances, binder element or tape 90 will act to prevent edge and end leakage of processing composition from the film unit during and subsequent to photographic processing.

Rupturable container 66 may be configured in similar fashion and will operate according to the general principals of the container described at 16 in connection with FIGS. 1-4.

- Container 62 is fixedly positioned and extends transverse to a leading edge of photosensitive laminate 66 whereby to effect unidirectional discharge of the container's contents 64 intermediate sheet 88 and surface 92 of blue-sensitive silver halide emulsion layer 68, upon application of compressive force to container 62. Thus, container 62, as illustrated in FIG. 5, is fixedly positioned and extends transverse to a leading edge of laminate 66 with its longitudinal marginal seal 94 directed toward the leading edge of surface 68. Container 62 is fixedly secured to laminate 66 by extension 96 of binder or tape 90 in combination with a separate retaining member such as tape 98 extending over a portion of the opposite wall of the container and a portion of laminate 66's surface.
- Sheet 88 is fixedly coupled to tape 98 extending transverse the leading edge of film unit 60 and is adapted to be superposed, subsequent to photoexposure of laminate 66, on and coextensive with surface 92 of blue-sensitive emulsion layer 68, at least during processing, to facilitate distribution of processing composition 64 upon compressive rupture of container 62 and unidirectional discharge of its contents intermediate surface 92 and superposed sheet 88.

Extension flap 30 of binder tape 90 may be of such area and dimension that upon, for example, manual separation of container 62 subsequent to distribution of the composition, from the remainder of the film unit 60, flap 96 may be folded over the edge of laminate 66 to facilitate maintenance of the composite structural integrity. Preferably, however, the film unit will be maintained intact subsequent to processing including retention of the exhausted container, the processing composition and sheet element in the spatial position assumed during processing. In such instance, the processing composition employed should possess the requisite adhesive capacity, in both fluid and dry states, to enhance the integrity and stability of the spatial arrangement assumed.

In general, in a particularly preferred embodiment, the processing composition 64 and/or sheet 88 when distributed will be sufficiently opaque to prevent further exposure of the film unit's silver halide emulsion or emulsions, by actinic radiation incident on sheet 88, during processing of the unit in the presence of radiation actinic to the emulsion or emulsions. Accordingly, the film unit detail may be processed, subsequent to exposure, in the presence of such radiation, in view of the fact that the silver halide emulsion or emulsions of the laminate may be appropriately protected from incident radiation, at one major surface by the opaque layer and layers 78 and at the remaining major surface by an opaque processing composition 64 and/or opaque sheet 88 as further described hereinafter. Note that, as before, processing is carried out by drawing the assembly 60 through processing rolls as at 100 and 102. As in the earlier embodiments, the binder tapes as at 90 also are opaque to prevent edge leakage of actinic radiation. The selected opaque layer or layers 78, however, should be one providing a background suitable for viewing the dye developer transfer image formed in the dyeable polymeric layer. In general, while substantially any permeable opaque layer may be employed, it is

preferred that it be selected so as not to interfere with the color integrity of the dye transfer image, as viewed by the observer, and, most preferably, a layer which is aesthetically pleasing to the viewer and does not provide a background noise signal degrading, or detracting 5 from, the information content of the image.

The opaque layer may comprise substantially any opacifying agent compatible with the photographic system, such as, for example, barium sulfate, zinc oxide, titanium dioxide, barium stearate, silver flake, silicates, 10 illumina, zirconium oxide, zirconium acetyl acetate, sodium zirconium sulfate, kaolin, mica, and the like, which may be distributed in a permeable polymeric matrix binder, such as, for example, gelatin, polyvinyl alcohol and the like. The opacifying capacity of the 15 opaque layer may be improved beyond that ordinarily obtained by the addition of an additional agent such as carbon black.

The opacifying agent dispersed in processing composition 64 may be any of the multiplicity of such agents 20 known in the art such as carbon black, iron oxide, titanium (III) oxide, titanium (III) hydroxide, and the like.

Film unit 60 is exposed to radiation actinic to photo-sensitive laminate 66 incident on the surface thereof. To provide for such exposure, sheet 88 is retained in a 25 position away from covering relationship with surface 68. Following exposure, the unit 60 is drawn through rolls 100 and 102 to effect superpositioning of sheet 88 contiguous to surface 92 of laminate 66 and to apply 30 suitable compressive pressure to container 62 with resultant distribution of processing composition 64.

Processing composition 64 permeates emulsion layers 68, 72 and 76 to initiate development of the latent images contained in the respective emulsions. The 35 cyan, magenta and yellow dye developers of these layers are immobilized, as a function of the development of their respective associated silver halide emulsions, preferably substantially as a result of their conversion from their reduced form to their relatively insoluble 40 and non-diffusible oxidized form, thereby providing image-wise distributions of mobile, soluble and diffusible cyan, magenta and yellow dye developer, as a function of the point-to-point degree of their associated emulsion's exposure. At least part of the image-wise distributions of mobile cyan, magenta and yellow dye developer transfer, by diffusion, to processing composition permeable polymeric layer 82, permeable spacer layer 84 and to polymeric acid layer 86 whereby solution 64 decreases in pH, as a function of neutralization, to a pH 45 at which the cyan, magenta and yellow dye developers, in the reduced form, are substantially non-diffusible, to provide thereby a stable multicolor dye transfer image viewable through dimensionally stable transparent layer 86. 50

It may be observed that in the structure of the film unit of FIGS. 5 and 6, the silver halide emulsion and the associated dye developer are formed within a singular binder. It should be appreciated that the structure may be formed wherein the dye developer layers are provided within a separate layer and binder. 55

Film units similar to that set forth in the drawings may be prepared, for example, by coating in succession, on a transparent cellulose triacetate film base:

1. the partial butyl ester of polyethylene/maleic anhydride copolymer prepared by refluxing for 14 hours, about 300 grams of high viscosity poly(ethylene/maleic anhydride), about 140 grams of

- n-butyl alcohol and about 1 cc. of 85% phosphoric acid to provide a polymeric acid layer approximately 0.75 mil. thick;
2. a solution of hydroxy propyl cellulose in water to provide a polymeric spacer layer approximately 0.075 mils. thick;
3. a 2:1 mixture, by weight, of polyvinyl alcohol and poly-4-vinylpyridine, at a coverage of approximately 600 mgs./ft.<sup>2</sup>, to provide a polymeric image-receiving layer approximately 0.40 mils. thick;
4. a layer of titanium dioxide dispersed in hydroxyethyl cellulose and coated at a coverage of about 1,200 mgs./ft.<sup>2</sup> of titanium dioxide and about 30 mgs./ft.<sup>2</sup> of hydroxyethyl cellulose;
5. a layer of gelatin coated at a coverage of about 200 mgs./ft.<sup>2</sup>;
6. a layer of the acrylic latex sold by Rohm and Haas Co., Philadelphia, Pa., under the trade designation Rhoplex AC-61 coated at a coverage of about 110 mgs./ft.<sup>2</sup>;
7. a layer of carbon black dispersed in hydroxyethyl cellulose coated at a coverage of about 150 mgs./ft.<sup>2</sup> carbon black and about 3.0 mgs./ft.<sup>2</sup> hydroxyethyl cellulose;
8. a layer of the cyan dye developer 1,4-bis-( $\beta$ [hydroquinonyl- $\alpha$ -methyl]-ethyl-amino)-5,8-dihydroxy-antraquinone and carbon black dispersed in gelatin and coated at a coverage of about 50 mgs./ft.<sup>2</sup> of dye, about 180 mgs./ft.<sup>2</sup> of carbon black and about 63 mgs./ft.<sup>2</sup> of gelatin;
9. a red-sensitive gelatino silver iodobromide emulsion coated at a coverage of about 120 mgs./ft.<sup>2</sup> of silver and about 22 mgs./ft.<sup>2</sup> of gelatin;
10. a layer of Rhoplex AC-61 coated at a coverage of about 80 mgs./ft.<sup>2</sup>;
11. a layer of the magenta dye developer 4-isopropoxy-2-[p-( $\beta$ -hydroquinonyl ethyl)-phenylazo]-naphthalene-1-ethoxy acetate dispersed in a green-sensitive gelatino silver iodobromide emulsion coated at a coverage of about 80 mgs./ft.<sup>2</sup> of dye, about 110 mgs./ft.<sup>2</sup> of silver and about 150 mgs./ft.<sup>2</sup> of gelatin;
12. a layer of the last-mentioned magenta dye developer dispersed in gelatin at a coverage of about 20 mgs./ft.<sup>2</sup> of dye and about 30 mgs./ft.<sup>2</sup> gelatin;
13. a layer of Rhoplex AC-61 coated at a coverage of about 110 mgs./ft.<sup>2</sup>;
14. a layer of the yellow dye developer 4-(p-[ $\beta$ -hydroquinonyl ethyl]-phenylazo)-3-(N-n-hexylcarboxamido)-1-phenyl-5-pyrazolone dispersed in gelatin and coated at a coverage of about 140 mgs./ft.<sup>2</sup> of dye and about 175 mgs./ft.<sup>2</sup> of gelatin;
15. a blue-sensitive gelatino silver iodobromide emulsion coated at a coverage of about 150 mgs./ft.<sup>2</sup> of silver and about 28 mgs./ft.<sup>2</sup> of gelatin; and
16. a layer containing 4'-methylphenyl hydroquinone dispersed in gelatin at a coverage of about 20 mgs./ft.<sup>2</sup> of 4'-methylphenyl hydroquinone and about 30 mgs./ft.<sup>2</sup> of gelatin.

A rupturable container comprising an outer layer of paper, an intermediate layer of lead foil and an inner liner or layer of polyvinyl chloride retaining an aqueous alkaline processing solution comprising:

|                                                                                                                                                    | 100  | cc.  | gms. |
|----------------------------------------------------------------------------------------------------------------------------------------------------|------|------|------|
| Water                                                                                                                                              | 11.2 |      |      |
| Potassium hydroxide                                                                                                                                | 3.4  |      |      |
| Hydroxyethyl cellulose (high viscosity) [commercially available from Hercules Powder Co., Wilmington, Delaware, under the trade name Natrasol 250] |      |      |      |
| N-benzyl- $\alpha$ -picolinium bromide                                                                                                             | 1.5  | gms. |      |
| Benzotriazole                                                                                                                                      | 1.0  | gm.  |      |
| Carbon black                                                                                                                                       | 6.4  | gms. |      |

and an opaque cellulose triacetate sheet may then be fixedly mounted on the leading edge, of each of the laminates, by pressure-sensitive tapes interconnecting the respective sheets, containers and laminates, such that upon application of compressive pressure to the container and superpositioning of the sheet, the container's contents will be distributed, upon rupture of the container's marginal seal, intermediate the cellulose triacetate sheet and the 4'-methylphenyl hydroquinone containing layer.

In accordance with the instant invention, film unit structures of the general designs described above advantageously may be fabricated incorporating low gel systems. As is described in U.S. Pat. No. 3,705,798 by the present inventors, such systems may be derived by incorporating select additions of water-soluble anionic polymeric materials, for instance, within the silver halide layers. Preferred materials for this purpose are the salts of polyvinyl hydrogen phthalate (PVHP). When added within appropriate gelatin supported layers, the additives permit the derivation of greater dye transfer densities and faster diffusion rates than can be obtained with like layers containing gelatin alone. The improved dye transfer performance, at least in part, derives from the fact that the combination permits one to use layers containing less matrix or carrier while still providing the desired physical properties such as viscosity that one could provide employing the gelatin alone. The employment of lesser amounts of carrier, for example, for the silver halide and color image-providing material, permits the deposition of thinner layers of same. This in turn evolves a system presenting less of a barrier to dye transfer. Additionally, improved image resolution is realized inasmuch as the available extent of laterally directed diffusion is more restricted. The addition of a water-soluble salt of PVHP to a gelatin silver halide solution after ripening also provides a decrease in fog level which in turn further contributes to dye transfer control and subsequent color quality of the transfer image.

It now has been determined that the addition of a water-soluble cellulose salt, preferably sodium cellulose sulfate (SCS), to the gelatin layers not only permits the fabrication of a low gel system, but also has no deleterious effects within the dye containing layers. For instance, in certain applications, gel/dye aggregates might otherwise be formed during post-production storage periods. The effectiveness of incorporating a water-soluble cellulose salt as the thickening agent permitting derivation of a low gel system within dye layers may be evidenced in the following examples.

The use of sodium cellulose sulfate as a gel reduction additive to a magenta dye transfer developer-gelatin layer permitted a change in the gel/dye (weight-to-weight) ratio from a value of 0.875 using a more typical additive such as a condensed naphthylene sulfonate to 0.600 where SCS is utilized. This represents a 31.4% reduction in the gelatin constituent. The formulation deriving this 0.600 gel-to-dye ratio was as follows:

7.20% 1:1 chrome complexed azo dye developer

|                                                                                                                                                         |
|---------------------------------------------------------------------------------------------------------------------------------------------------------|
| 0.21% "Lomar D" a condensed naphthylene sulfonate used here as a dispersing agent. (Commercially available from Nopco Chemical Co., Newark, New Jersey) |
| 4.32% inert gelatin                                                                                                                                     |
| 0.18% sodium cellulose sulfate                                                                                                                          |
| 88.09% H <sub>2</sub> O                                                                                                                                 |

A low gel system operating in conjunction with a yellow diffusion transfer dye developer has been prepared wherein the gelatin-to-dye ratio has been lowered from a typical value of 0.708 using Lomar D as an additive to 0.400 using SCS. This alteration represents a 43.0% reduction in the gelatin constituent. The formulation providing for this 0.400 gelatin/dye system was as follows:

|                                                       |
|-------------------------------------------------------|
| 7.20% 1:1 chrome complexed azo methine dye developer  |
| 0.36% Lomar D (supra, utilized as a dispersing agent) |
| 2.88% inert gelatin                                   |
| 0.17% sodium cellulose sulfate                        |
| 89.39% H <sub>2</sub> O                               |

A low gel system operating in conjunction with a cyan dye developer has been prepared wherein the gelatin-to-dye ratio has been lowered from a typical value of 1.46 using Lomar D as an additive to a value of 0.500 using SCS. This alteration represents a 66.0% reduction in the gelatin constituent. The formulation providing for this 0.500 gelatin/dye system was as follows:

|                                                       |
|-------------------------------------------------------|
| 6.50% copper phthalocyanine dye developer             |
| 0.19% Lomar D (supra, utilized as a dispersing agent) |
| 3.25% inert gelatin                                   |
| 0.20% sodium cellulose sulfate                        |
| 89.90% H <sub>2</sub> O                               |

An "ultra-low gel system" also is available in accordance with the present invention. The following formulations have been developed to evolve a gel-dye (weight-to-weight) ratio of 0.300. For example, the following formulation provided an ultra-low gel system for a magenta dye transfer developer:

|                                                       |
|-------------------------------------------------------|
| 8.50% 1:1 chrome complexed azo dye developer          |
| 0.26% Lomar D (supra, utilized as a dispersing agent) |
| 2.55% inert gelatin                                   |
| 0.08% sodium cellulose sulfate                        |
| 88.61% H <sub>2</sub> O                               |

An ultra-low gel system operating in conjunction with a yellow diffusion transfer dye developer has been prepared having the following formulation:

|                                                       |
|-------------------------------------------------------|
| 8.50% 1:1 chrome complexed azo methine dye developer  |
| 0.42% Lomar D (supra, utilized as a dispersing agent) |
| 2.55% inert gelatin                                   |
| 0.08% sodium cellulose sulfate                        |
| 88.45% H <sub>2</sub> O                               |

An ultra-low gel system operating in conjunction with a cyan dye developer has been prepared with the following formulation:

|                                                       |
|-------------------------------------------------------|
| 7.50% copper phthalocyanine dye developer             |
| 0.23% Lomar D (supra, utilized as a dispersing agent) |
| 2.25% inert gelatin                                   |
| 0.08% sodium cellulose sulfate                        |
| 89.95% H <sub>2</sub> O                               |

In appropriate circumstances, the composite film unit structure may be provided wherein the gelatino silver halide layers and dye transfer developer-gelatin layers are provided as discrete layers or depositions. With such an arrangement, select ones of the gelatino silver halide layers may incorporate a salt of PVHP, while associated dye layers will contain the water-soluble cellulose salt as described herein. Alternately, both the halide and the dye material dispersions may incorporate the water-soluble cellulose salt as a low gel system additive. 10

The additives described herein may be utilized in conjunction with any of a broad variety of diffusion transfer film unit structures including the integral structure shown in the drawings as well as structures described in certain of the reference patents wherein the image-receiving element is stripped from the photosensitive element following an appropriate interval of imbibition.

Since certain changes may be made in the above products and processes without departing from the scope of the invention herein involved, it is intended that all matter contained in the above description or shown in the accompanying drawings shall be interpreted as illustrative and not in a limiting sense. 20

We claim:

1. A photographic film unit, adapted to be exposed and processed to produce a color diffusion transfer image, comprising:

a plurality of layers including at least one composite photosensitive unit comprising a light-sensitive silver halide layer and, in contiguous planar relationship thereto, a layer comprising a select associated diffusion transfer dye image-forming material dispersed in a matrix comprising gelatin and sodium 30

35

cellulose sulphate; receptor means including a layer adapted to receive diffusion transfer dye-image forming material diffusing thereto as a function of the point-to-point degree of said photosensitive unit's exposure to incident actinic radiation; means incorporated with said film unit for selectively providing processing composition intermediate said receptor means and said plurality of layers; and means defining a dimensionally stable support for said plurality of layers.

2. The photographic film unit of claim 1 wherein said sodium cellulose sulfate is present in an amount effective to provide for a weight-to-weight ratio, respectively, of said gelatin to said dye image-providing material of less than about 0.6. 15

3. The photographic film unit of claim 1 wherein said plurality of layers comprise a first composite photosensitive unit including a blue-sensitive gelatino silver halide emulsion layer and a layer containing a gelatin carried yellow dye image-forming material, a second composite photosensitive unit including a green-sensitive gelatino silver halide emulsion layer and a layer containing a gelatin carried magenta dye image-forming material; and a third composite photosensitive unit including a red-sensitive gelatino silver halide emulsion layer and a layer containing a gelatin carried cyan dye image-forming material. 25

4. The photographic film unit of claim 3 wherein said gelatin within a said dye-forming material containing layer is present in a weight-to-weight ratio with respect to said dye image-forming material of less than about 0.6. 30

\* \* \* \* \*

40

45

50

55

60

65